

Dec. 1, 1936.

J. F. JOSEPH

2,062,317

ROLL

Filed April 3, 1935



Fig. 1.

Inventor

*John F. Joseph*

By

*Murray and Zugelter*  
Attorneys

## UNITED STATES PATENT OFFICE

2,062,317

## ROLL

John F. Joseph, Cincinnati, Ohio, assignor to The  
Cincinnati Rubber Manufacturing Company,  
Norwood, Ohio, a corporation of Ohio

Application April 3, 1935, Serial No. 14,537

12 Claims. (Cl. 92—49)

This invention relates to a roll of the type employed in paper making machines and with which a doctor is commonly utilized.

An object of the invention is to provide a roll of this kind adapted to resist wear and the adhesion of paper and paper pulp and the like to its surface.

Another object is to provide such a roll which is adapted to resist the wear ordinarily resulting from a doctor bearing against the roll and at the same time which roll is so formed as to obviate injury to the doctor itself.

Another object is to produce a roll of the kind described cheaply and efficiently.

15 These and other objects are attained by the means described herein and illustrated in the accompanying drawing, in which:

The figure is an elevational view, with parts broken away, of a roll produced according to the present invention.

Heretofore rolls of the class herein considered, have been manufactured of various materials, including wood, granite, and other materials upon which hard smooth surfaces were capable of being produced. It was necessary, however, to keep wood rolls constantly wet, even during the period when the machinery with which they were associated, was not in use, so as to avoid splitting of the rolls. The granite rolls were objectionable 30 because of the great expense involved in producing granite rolls of the large size necessary in modern paper machinery. Furthermore, there has been produced heretofore rolls comprising a body formed of a binder, such as rubber having incorporated therein crystalline or rock particles for forming a firm working surface adapted to avoid the adhesion of paper pulp and the like thereto. Rolls such as the latter have, however, possessed this disadvantage, that their use resulted in undue wear on the doctor commonly utilized with such rolls when employed as "top rolls" in paper making machinery.

Another marked disadvantage noted in connection with rolls having incorporated therein crystalline particles such as granite, has been the formation of cracks in the roll due to lack of effective bonding between such smooth-surfaced particles and the binder. Similar undesirable results accompany the use of fibrous particles, sometimes utilized in the roll in the manner of the crystalline particles, such results again being due to lack of an integral and cohesive union of the binder and the particles.

The present invention obviates the disadvantages enumerated above by providing a roll

formed with a binder, such as rubber, having irregular cellular particles, such as particles of blast furnace slag, incorporated therein. The roll so formed need not be constantly treated as was necessary with wooden rolls and may be 5 readily and efficiently as well as cheaply manufactured, as compared with the older type of granite roll. Finally, the roll of this invention, due to the inclusion of slag of the kind described, which is considerably less abrasive than materials heretofore employed, reduces wear on the doctor employed with top rolls.

In greater detail, and with reference to the drawing: The roll of this invention may comprise a core 5, preferably metallic, and enlarged 15 as at 6 along that portion upon which the roll proper is to be formed. The body 7 of the roll of this invention is formed of a hard rubber or ebonite compound, which serves as a binder. Incorporated in the binder, throughout the surface 20 thereof and preferably throughout the whole body of the binder, are particles of slag 8, blast furnace slag having been found particularly effective for the present purpose. An analysis of this slag has disclosed its characteristics as follows:

|                  | Per cent |
|------------------|----------|
| Silicon di-oxide | 36.8     |
| Aluminum oxide   | 10.43    |
| Calcium oxide    | 32.5 30  |
| Magnesium oxide  | 14.100   |
| Iron             | 1.52     |
| Manganese        | .500     |
| Sulphur          | 1. 35    |

This analysis, however, it should be understood, is subject to wide variation, and is set forth merely as illustrative.

In the drawing, a portion only of the roll has been shown as provided with the particles 8 but it is to be understood that these are incorporated throughout the total surface or body of the binder. The roll of this invention may be produced by any suitable means or process, as will be understood. However, it has been found that an 45 efficient manufacturing process consists in turning the core 5 upon a lathe and applying the resilient material or rubber to the enlarged portion 6, while said material is in a plastic condition. During the application of the rubber, the 50 slag 8 is progressively incorporated in the plastic binder, the latter and the slag being of substantially the same proportion as to weight. An efficient method of combining the plastic binder and the slag is to masticate the two together before

the application thereof to the core. The body of the roll thus formed is subsequently cured. Thereafter the surface of the roll body is ground to produce a surface that is uniform and smooth thereby eliminating any projecting particles or points thereon. It is to be noted that the particles 8 being of cellular structure throughout, are not worn smooth by subsequent regrindings of the roll but rather additional minute apertures and 10 pits appear on the surfaces of the particles, thereby aiding in maintaining the roll's distinctive property of avoiding paper adhesion.

As above indicated, the peculiar quality of the blast furnace slag imparts to the roll the desirable 15 wear resistant character and at the same time minimizes a frictional wearing away of the doctor employed therewith. The peculiar surface quality of the roll whereby the adhesion thereto of paper in the process of manufacture is avoided, has already been referred to. However, other materials 20 possessing a cellular structure, such as cinders, might be used for the slag particles 8. Materials of this nature possess irregularities of form and surface whereby they are peculiarly adapted 25 to be keyed or locked permanently in the binder.

What is claimed is:

1. A roll comprising a resilient binder and slag particles incorporated in the binder throughout the surface of the roll.
2. A roll comprising a rubber binder and slag particles incorporated in the binder throughout the surface of the roll.
3. A roll comprising a rubber binder and particles of blast furnace slag incorporated in the binder throughout the surface of the roll.
4. A roll comprising a rubber binder and particles of blast furnace slag incorporated in the surface and body of the binder.

5. A roll for paper machinery or the like, and comprising a core, and a roll body attached to the core and consisting of a rubber binder having slag particles incorporated therein throughout the surface thereof for providing a wear-resistant roll surface adapted to minimize injury to the doctor normally utilized with rolls of the kind described.

6. A roll for paper machinery or the like and comprising a metal body, the outside covering of which consists of a rubber binder, having particles of blast furnace slag, incorporated therein for providing a wear resistant surface, the latter being adapted to avoid adhesion of paper and paper pulp thereto and to minimize abrasion to the doctor normally utilized with rolls of the kind described.

7. A roll comprising a rubber binder and particles of blast furnace slag incorporated throughout the binder and of substantially the same proportion as to weight as that of the binder.

8. A roll comprising a binder with slag-like cellular particles incorporated therein.

9. A roll comprising a binder having incorporated therein slag-like irregularly-shaped particles of cellular structure.

10. A roll comprising a binder with slag-like irregularly-shaped particles incorporated therein.

11. A roll comprising a binder having incorporated therein particles of the class of slag and cinders.

12. A roll for paper machinery or the like and comprising a metal body the outside covering of which consists of a rubber binder having particles of the class of slag and cinders incorporated therein for providing a wear-resistant surface, said particles being of substantially the same proportion as to weight as that of the binder.

JOHN F. JOSEPH.